

## UNITED STATES PATENT OFFICE

2,311,498

## AVIATION FUEL

Alexis Voorhies, Jr., Baton Rouge, La., assignor,  
by means assignments, to Standard Catalytic  
Company, a corporation of Delaware

No Drawing. Application September 16, 1939,  
Serial No. 295,257

9 Claims. (Cl. 44-80)

This invention relates to aviation fuel and is more particularly concerned with a method of preparing an aviation fuel rich in aromatics having a high octane number and a high net heating value.

Recently there has been a substantial increase in the demand for aviation fuels of octane numbers in excess of 90 by the A. S. T. M. method and of 92 or more by the Army method. In addition to the requirement that the octane number must be a certain minimum it is also specified, among other things, that the lower or net heating value of the fuel shall be at least 18,500 B. t. u. per pound.

The lower or net heating value is determined by the following formula:

$$H - w \times 1050$$

where  $H$  is the higher or gross heating value of the fuel in B. t. u. per pound, and  $w$  is the weight in pounds of water per pound of fuel.

The higher or gross heating value is determined in accordance with A. S. T. M. method D-240-27. The weight in pounds of water per pound of fuel is determined in accordance with the method described in "Determination of Carbon and Hydrogen in Gasoline and other Volatile Liquids," Industrial and Engineering Chemistry (analytical edition), volume 9, No. 7, July 15, 1937.

I have found that an aviation gasoline should have a hydrogen content of at least 13.5% in order that the lower heating value will be at least 18,500 B. t. u. per pound. I have also found that many processes by which aviation gasolines of the required octane number can be prepared produce gasolines in which the hydrogen content is appreciably below 13.5% and consequently the lower heating value is below the required minimum of 18,500 B. t. u. per pound.

One particularly suitable method for preparing aviation gasolines of high octane number is a process of catalytic reforming in the presence of substantial quantities of added hydrogen carried out under such conditions of time, temperature, pressure and feed rate that there is a substantial net production of free hydrogen in the process. The term "catalytic reforming" wherever used in the specification and claims shall be understood to mean any process of subjecting materials consisting essentially of hydrocarbons substantially boiling in the gasoline range to heat treatment at a temperature in excess of 500° F. and in the pres-

ence of catalysts to produce dehydrogenated or otherwise chemically reconstructed product, for example of anti-knock characteristics superior to those of the starting material, with or without an accompanying change in molecular weight. By the term "chemically reconstructed" is meant something more than the mere removal of impurities or ordinary finishing treatments. The term catalytic reforming shall be understood to include, but not by way of limitation, reactions such as dehydrogenation, aromatization or cyclization, desulfurization, alkylation and isomerization, all or some of which may occur to a greater or lesser extent during the process.

It is observed that in catalytic reforming in the presence of hydrogen there is a substantial formation of aromatic hydrocarbons. While these aromatics are characterized by high octane number and have other characteristics which make them desirable for use in aviation fuel, they are also characterized by low hydrogen content which is unfavorable from the standpoint of high net heat of combustion. The problem therefore is to find some way to take advantage of the desirable characteristics of aromatic hydrocarbons and to offset their deficiency in hydrogen.

The present invention therefore has for its principal object the provision of a process by which an aromatic aviation fuel of high octane number and high net heating value may be produced. The nature of the process and the manner in which it is carried out will be fully understood from the following description.

A hydrocarbon oil of relatively low octane number and having a boiling range between say 100 and 500° F. is subjected to catalytic reforming in the presence of hydrogen. The hydrocarbon oil may be derived from any source and it is immaterial whether it is paraffinic, naphthenic, aromatic, olefinic or contains high or low sulfur content. The oil, preferably in admixture with hydrogen or a gas rich in free hydrogen, is heated to a temperature between 850 and 1050° F. under a pressure between atmospheric and 500 lbs. per square inch, preferably between 50 and 300 lbs. per square inch and is then passed over a catalyst which promotes reforming. Many different catalysts may be used but especially suitable ones are mixtures of aluminum oxide and oxides of metals of the IV, V, VI and VIII groups of the periodic system, particularly molybdenum, chromium, tungsten, vanadium, cobalt and nickel. These

catalysts may contain from 1 to 50% or more of the active metal oxide, and may be prepared in several different ways, i. e. by mechanical mixing of the ingredients, by impregnating the aluminum oxide with a solution of the metal salt and then heating to convert the metal salt to the oxide, or by co-precipitating aluminum hydroxide and the hydroxide of the active metal from a solution containing soluble salts of the two.

The quantity of gas containing hydrogen which is passed with the oil over the catalyst is preferably between 1000 and 4000 cubic feet per barrel of oil and this gas should contain from 20 to 90 mol per cent of free hydrogen. The rate at which the oil is passed over the catalyst is preferably between 0.3 and 3.0 volumes of liquid oil per volume of catalyst per hour.

The passage of oil and hydrogen over the catalyst is continued until (1) the octane number of the liquid product produced, as indicated by the aniline point thereof, falls below the desired level or (2) there ceases to be a net production of free hydrogen in the reaction, whichever of these things occurs first. With most of the catalysts mentioned above, this time may vary from 3 to 6 hours or more. At the end of this time or cycle, it is necessary to regenerate the activity of the catalyst and the manner in which this can be done will be explained below.

The products leaving the reaction zone which consist of hydrocarbon vapors and hydrogen are passed through a cooler, and then into a separator wherein liquid and gaseous products are separated.

The gaseous products which contain substantial quantities of free hydrogen are removed and may be recycled directly to the reaction zone to provide the gas rich in free hydrogen required therein, or a portion or all of them may first be scrubbed with oil or otherwise treated to remove some of the hydrocarbon constituents and thereby increase the concentration of hydrogen therein. It will be understood that once the process has started up it will not be necessary to add hydrogen from an extraneous source because the hydrogen produced in the process is sufficient to maintain the required concentration in the recycle gases.

The liquid products are removed from the separator, pressure is released thereon whereby further quantities of gas are evolved, and these gases are removed from the system. The products which still remain liquid are passed into a fractionating and stabilizing tower and a fraction boiling in the aviation fuel range is separated therefrom. This product will have a substantially higher octane number than the feed stock, and, unless the conditions of operation have been so selected and held within such narrow limits as to retard the formation of aromatics, will be substantially richer in aromatic hydrocarbons than the feed stock. In most cases, the aromatic content of this product will range between 20 and 55%. However, in such cases, the hydrogen content will be appreciably below the 13.5% minimum necessary to insure a lower net heating value of at least 18,500 B. t. u. per pound.

Returning to the regeneration referred to above, when the catalyst requires regeneration the flow of oil and hydrogen is stopped, the reaction chamber is purged of oil by passing inert gases or steam therethrough and then hot inert gases containing regulated quantities of air or oxygen are passed over the catalyst whereby the coke and carbonaceous contaminants deposited

thereon are removed by combustion. The quantity of gases passed through the catalyst may vary from 1000 to 3000 volumes of gas per volume of catalyst per hour. The gases are heated to a temperature of 600 to 900° F. and care should be taken that the highest temperature in the reaction zone does not exceed about 1200° F. One method of temperature control is through the oxygen concentration of the regeneration gases. For example, at the start of the regeneration when combustion is rapid the concentration of oxygen may be low such as 0.3% and as the regeneration proceeds the quantity may be increased to 10 or even 21%.

The flow of regenerating gases is ordinarily continued until there is no longer a consumption of oxygen therefrom. This will indicate that no further combustible material remains on the catalyst. After regeneration the catalyst may be used again in a reaction cycle and alternate reaction and regeneration cycles may be carried out an indefinite number of times.

Following fractionation and if necessary re-running, the product of the above process is blended with a sufficient quantity of a hydrocarbon having an octane number at least as high as that of the product and a hydrogen content substantially above 13.5% to bring the hydrogen content of the entire mixture up to or above 13.5%. Suitable hydrocarbons for this purpose are isopentane and isobutane or isopentane which have been alkylated with normally gaseous olefins. These hydrocarbons may be obtained from any source. An especially convenient source of isopentane is the feed stock itself which may be depentanized prior to the catalytic reforming treatment, and the pentane so obtained isomerized in any known manner, such as by heating in the presence of aluminum chloride and hydrogen chloride. Part or all of the isopentane so obtained may be blended with the reformed product. It will be understood of course that the quantity of isopentane added should not be sufficient to make the final blend too volatile.

The quantity of isopentane that must be added will naturally depend upon the hydrogen content of the reformed fuel and the volatility desired in the final fuel. In general I have found that quantities of isopentane between 5 and 15% may be used with satisfactory results.

The following examples illustrate how the invention is applied:

#### Example 1

55 A light naphtha derived from an East Texas crude and having the following characteristics:

|                            |      |
|----------------------------|------|
| Gravity, A. P. I.          | 63.3 |
| Aniline point, °F.         | 131  |
| Octane number, A. S. T. M. | 59.2 |
| Bromine number             | 1    |
| Initial boiling point, °F. | 117  |
| Final boiling point, °F.   | 345  |
| Percent aromatics          | 15   |

60 is subjected to catalytic reforming in the presence of hydrogen under the following conditions:

|                                       |      |
|---------------------------------------|------|
| Pressure, lbs./sq. in.                | 200  |
| Temperature, °F.                      | 950  |
| Recycle gas rate, cu. ft./bbl. oil    | 2800 |
| Percent H <sub>2</sub> in recycle gas | 73   |
| Oil feed rate, v./v./hr.              | 0.5  |
| Catalyst                              |      |

65 Activated alumina and molybdenum oxide  
70 Length of cycle, hours

A gasoline boiling in the aviation fuel range is separated from the product of this treatment and treated with 5#/bbl. of 98% sulfuric acid. This treated gasoline has the following characteristics:

|                                        |       |
|----------------------------------------|-------|
| Gravity, °A. P. I.                     | 55.3  |
| Aniline point, °F.                     | 62    |
| Octane number, A. S. T. M.             | 79.6  |
| +3 cc. lead.                           | 90.5  |
| +6 cc. lead.                           | 93.6  |
| Bromine number                         | 8     |
| Army gum, mgs.                         | 1.4   |
| Acid heat, °F. A. S. T. M.             | 11    |
| Reid V. P., lbs./sq. in.               | 5.9   |
| Initial boiling point, °F.             | 15    |
| Per cent @ 167 °F.                     | 127   |
| Per cent @ 212 °F.                     | 22.0  |
| Per cent @ 293 °F.                     | 52.0  |
| Final boiling point, °F.               | 93.0  |
| Yield on feed, vol. per cent           | 79    |
| Gross heat of combustion, B. t. u./lb. | 19548 |
| Net heat of combustion, B. t. u./lb.   | 18333 |
| Hydrogen content, per cent             | 12.8  |
| Per cent aromatics                     | 42    |

20% and 30% respectively of an alkylate prepared by alkylating isobutane with butylenes is added to the above fuel and the characteristics of the blend are then as follows:

|                                     | Alkylate<br>20% | Added<br>30% |
|-------------------------------------|-----------------|--------------|
| Gravity °A. P. I.                   | 57.7            | 59.3         |
| Octane number A. S. T. M.           | 82.4            |              |
| +3 cc. lead.                        | 92.7            |              |
| +6 cc. lead.                        | 95.0            |              |
| Initial boiling point °F.           | 116             | 118          |
| Percent @ 167 °F.                   | 16              | 14.5         |
| Percent @ 212 °F.                   | 49.5            | 48.5         |
| Percent @ 293 °F.                   | 94.0            | 95.5         |
| Final boiling point °F.             | 317             | 314          |
| Gross heat of combustion B.t.u./lb. | 19744           | 19843        |
| Net heat of combustion B.t.u./lb.   | 18476           | 18528        |
| Hydrogen content percent            | 13.4            | 13.9         |

It will be seen from the above example that the net heat of combustion can be increased from 18,333 to at least 18,500 B. t. u./lb. with an actual increase in the octane number.

#### Example 2

To another portion of the same acid-treated hydroformed naphtha is added 11% of isopentane and it then has the following characteristics:

|                                        |        |
|----------------------------------------|--------|
| Gravity °A. P. I.                      | 58.4   |
| Gross heat of combustion, B. t. u./lb. | 19,720 |
| Net heat of combustion, B. t. u./lb.   | 18,462 |
| Hydrogen content, per cent             | 13.3   |

It will be seen from the above example that the addition of about 15% of isopentane to the base stock will increase the net heat of combustion to at least 18,500 B. t. u./lb.

While the above description of the invention has been made with particular reference to an aviation fuel prepared by a process of catalytic reforming in the presence of hydrogen, it will be understood that the method of increasing the net heat of combustion to at least 18,500 B. t. u./lb. is equally applicable to aviation fuels prepared by other processes, such as catalytic cracking, catalytic reforming, thermal cracking, thermal reforming and the like.

It will also be understood that this method is equally applicable to raising the net heating value to any other figure within reasonable limits of 18,000 B. t. u. per pound and that there is a definite minimum hydrogen content which corresponds to each particular lower net heating value. Moreover the relationship between heat of combustion and hydrogen content is a straight line relationship so that it is a simple matter to determine what the hydrogen content should be when the minimum lower net heating value has been set. The following table shows the hydrogen content corresponding to certain lower net heating values:

| Per cent hydrogen<br>by weight | Lower net heating<br>value B. t. u. per pound |
|--------------------------------|-----------------------------------------------|
| 9.1                            | 17,500                                        |
| 10.2                           | 17,750                                        |
| 11.3                           | 18,000                                        |
| 12.4                           | 18,250                                        |
| 13.5                           | 18,500                                        |
| 15.7                           | 19,000                                        |

These figures when plotted fall on a straight line so that intermediate values may be readily determined. In using such a plot due allowance should of course be made for experimental deviations from the curve.

This invention is not limited by any theories of the mechanism of the reactions nor by any details which have been given merely for purposes of illustration but is limited only in and by the following claims in which it is intended to claim all novelty inherent in the invention.

I claim:

1. The method of increasing the net heat of combustion of an aviation fuel containing between 20 and 55% of aromatic hydrocarbons to at least 18,500 B. t. u. per pound without substantially affecting the octane number of said fuel which comprises adding thereto a sufficient quantity of a hydrocarbon having an octane number at least equal to that of the fuel and a hydrogen content in excess of 13.5% to bring the hydrogen content of the mixture to at least 13.5%.

2. Method according to claim 1 in which the hydrocarbon added to the fuel is isopentane.

3. Method according to claim 1 in which the hydrocarbon added to the fuel is an alkylate of isobutane and a normally gaseous olefin.

4. Method according to claim 1 in which the hydrocarbon added to the fuel is an alkylate of isopentane and a normally gaseous olefin.

5. The method of preparing an aviation fuel having an A. S. T. M. octane number with 3 ccs. of tetraethyl lead in excess of 90 and a net heat of combustion of at least 18,500 B. t. u. per pound which comprises adding to a hydrocarbon oil containing between 20 and 55% of aromatic hydrocarbon, consisting essentially of hydrocarbons boiling in the aviation fuel range and prepared by a process of catalytic reforming in the

presence of hydrogen carried out under such conditions that there is a net production of free hydrogen in the reaction, a minor quantity of a hydrocarbon having an octane number at least equal to that of said hydrocarbon oil and a hydrogen content in excess of 13.5% by weight sufficient to bring the hydrogen content of the mixture to at least 13.5% by weight.

6. Method according to claim 5 in which the hydrocarbon added is isopentane.

7. Method according to claim 5 in which the hydrocarbon added is an alkylate of isopentane and a normally gaseous olefin.
8. Method according to claim 5 in which the hydrocarbon added is an alkylate of isobutane and a normally gaseous olefin.

9. Method according to claim 5 in which the hydrocarbon added is isopentane and the quantity thereof added is between 5 and 15% by volume.

ALEXIS VOORHIES, JR.